

## UNITED STATES PATENT OFFICE

MAX FECHTER, OF PHILADELPHIA, PENNSYLVANIA

## VARNISH

No Drawing.

Application filed May 6, 1925. Serial No. 28,504.

This invention relates to varnishes, and the principal object of the invention is to provide a varnish having characteristics both of spirit and oil varnishes and being adapted 5 for application to a wood or other surface without the usual priming coat of shellac or other spirit varnish.

As a characteristic example of my improved varnish and the method of manufacturing, the procedure may be as follows: I may first form a solvent consisting of denatured alcohol and oxalic acid in the proportions approximately of one ounce of oxalic acid to each quart of alcohol. To this 10 solvent I add gum sandarac (juniper gum) and gum mastic, two parts by weight of the sandarac and one part of the mastic. The proportion of the mixed gums to the solvent may vary to some extent, but for general 15 purposes I have found two and one-half pounds of the mixed gums to one gallon of the solvent satisfactory. The mixture is then heated in a water bath until the gum has been entirely dissolved, after which the solution 20 is allowed to settle until clear and the clear liquid drawn off. Denatured alcohol may be added to make up the losses in the heating operation. For purpose of this description, I will designate this solution as "solution 25 No. 1".

I then form a mixture of fused gum dammar, hard oil finish and turpentine, employing equal parts of these materials, and this mixture is heated in a water bath until the 30 gum has entirely dissolved and the mixture becomes thoroughly homogeneous. This solution is allowed to stand until the insoluble residue has settled, after which the clear solution is drawn off. This solution I may designate as "solution No. 2". The hard oil finish may be formed by boiling 35 parts of linseed oil with 3 parts red lead and 1 part white vitriol.

Solutions Nos. 1 and 2 are then mixed together, preferably in the proportions of three

parts of No. 1 to one part No. 2, and are boiled in a water bath for approximately one-half hour and are again allowed to stand until any insoluble residue has settled out, after which the clear liquid solution constituting a mixture of solutions Nos. 1 and 2 is drawn off. This combined solution I may designate as "solution No. 3".

A fourth solution is then formed as follows: Dissolve in 1 quart of wood alcohol 50 of 95% proof,  $\frac{1}{2}$  ounce of pyroxylin and  $\frac{1}{4}$  ounce of camphor, and add to the solution 55 8 ounces of ether. The pyroxylin and camphor may be replaced by celluloid chips in amount approximately 3 ounces. To the resulting solution, I then add sassafras oil, 60 approximately one part of sassafras oil to two parts of the said solution, and the resultant mixture, which I may term "solution No. 4", is added to solution No. 3, approximately 65 one part of solution No. 4 to sixteen parts of solution No. 3, this mixture constituting the final product.

The product constitutes a hard quick drying varnish for inside work which may be 70 sprayed onto wood or other surface without the necessity of first priming the surface with shellac or the like, this being possible by reason of the fact that the varnish combines the characteristics both of shellac, or similar 75 spirit varnish, and of an oil varnish, and this varnish may be rubbed with pumice and water and polished and brought to a finish in less time than varnishes now generally used.

It will be understood that I do not desire 80 to limit myself to the exact ingredients and proportions herein set forth, and that I consider my invention as covering not only the specific varnish described but any varnish having similar characteristics and compounded in substantially the same manner with materials the equivalents of the materials herein set forth.

I claim:

1. The process that includes forming a 90

spirit varnish including oxalic acid, forming an oil varnish, mixing said varnishes, forming an alcohol solution of pyroxylin including sassafras oil, and mixing the last-named solution with the mixed varnishes.

- 5 2. The process that consists in forming a spirit varnish containing gum sandarac and gum mastic in a solvent of alcohol containing oxalic acid, mixing therewith an oil varnish  
10 containing fused gum dammar, hard oil finish and turpentine, and adding to said mixture an alcohol solution of pyroxylin.

**MAX FECHTER.**